

Nov. 20, 1934.

S. C. FULTON

1,981,824

## PROCESS OF PRODUCING RESINS OF PETROLEUM ORIGIN

Filed Oct. 30, 1931



*Stewart C. Fulton* Inventor

୩୩୫

W. E. Currie attorney

## UNITED STATES PATENT OFFICE

1,981,824

PROCESS FOR PRODUCING RESINS OF  
PETROLEUM ORIGINStewart C. Fulton, Elizabeth, N. J., assignor to  
Standard Oil Development Company, a corpo-  
ration of Delaware

Application October 30, 1931, Serial No. 572,058

4 Claims. (Cl. 260—2)

This invention relates to the production of synthetic resins from cracked tar-oils of petroleum origin and certain other petroleum distillates by condensation by means of chlorination and will be understood from the following description when read in conjunction with the drawing, which is a semi-diagrammatic side elevation, partly in section, of a suitable apparatus.

Cracked tar of petroleum origin obtained in liquid or vapor phase cracking, or any similar process involving cracking, is used as the preferred raw material for the production of resins. The tar which may have a gravity of, say, 10°-11° A. P. I., is first subjected to distillation, preferably under vacuum, to remove the oily components overhead. If a high vacuum, for example, 1 mm. mercury, is used, the oily components will distill over between the approximate temperatures of 300° F. to 660° F. corresponding to about 600° F., and about 1100° F. respectively at atmospheric pressure. However, it is not necessary to use such an extreme vacuum, but less vacuum with or without steam or other distillation aid may also be used and the distillation 25 may even be carried out under atmospheric pressure using steam or other gaseous agent as carrier. Usually about 85% of the tar is obtained as distillate.

The distillate is then chlorinated preferably by bubbling chlorine through it slowly. The temperature at which the chlorination is carried out may be ordinary room temperature or it may be somewhat higher, say up to 150° F., depending on the viscosity of the distillate. The product to 35 be chlorinated is preferably agitated while the chlorine is bubbled through it. The chlorination is continued until 10 to 15% of chlorine is absorbed, although it may be interrupted earlier or may be carried out further, depending on the product desired. The amount of chlorine absorbed may be determined by any of the known analytical methods, or it may be roughly estimated by the increase of weight of the product. The chlorinated product is then heated in a still 40 up to a temperature of about 660° F., first under atmospheric pressure, then under vacuum, the final step in the heating being preferably carried out under 1 mm. mercury pressure and at a temperature up to 660° F. The heating simultaneously removes as overhead products the chlorine in the form of hydrochloric acid and the oily products. Only traces of chlorine are found in the hydrocarbon material carried overhead and in the residue.

50 The bottoms remaining in the still is cooled

down to about 200° F. and then agitated with about three times its weight of a selective solvent for resin such as light petroleum hydrocarbon distillate (naphtha) to extract the resinous product. For example, the volatile petroleum hydrocarbon solvent known in commerce as "Varsol" 60 may be used for this purpose. This has the following specifications:

|                           |             |    |
|---------------------------|-------------|----|
| Color (Robinson) -----    | +22         | 65 |
| % off at 350° F. -----    | 55% minimum |    |
| % off at 392° F. -----    | 95% minimum |    |
| Final boiling point ----- | 410° F.     |    |
| Abel flash -----          | 100° F.     |    |
| Passes doctor test.       |             | 70 |

Although the solvent described is preferred, it will be understood that the present invention is in no way limited thereto.

Instead of using agitation the still bottoms may be refluxed with the hydrocarbon solvent. In either case the solution is separated from the hydrocarbon insoluble material, the amount of which varies from 0% to 50% of the weight of the bottoms. The separation is effected by settling and decantation or by filtration, or by other methods of separation known in the art. The hydrocarbon solvent is then removed from the dissolved resin by distilling the solution under atmospheric pressure or under slight vacuum, leaving as distillation residue the final resin 85 product. When a light-colored resin is required the solution in "Varsol" or naphtha is acid-treated before the final distillation step.

The concentration of the sulfuric acid used for this purpose is 95% more or less. The amount of the acid will be regulated according to the desired color of the final resin, and may vary within wide limits, say from 10% to 50% of the resinous material dissolved in the solvent. The acid sludge is separated and the solution is neutralized, either by contacting with fine clay or by washing with water or dilute alkali. The acid treated and neutralized solution is distilled to remove the naphtha from the resin, if a solid resin is required.

The yield of resin is on the average 15% of the tar distillate and will depend upon the degree of chlorination. The more thorough the chlorination, the higher will be the softening point of the resin. The latter is above about 80° F. and usually between 140° and 225° F. as determined by the ball and ring method. Increased chlorination, however, also increases the hydrocarbon insoluble material and consequently de-

100  
110

creases the yield. The final condensed resin is an unsaponifiable solid, odorless and tasteless, and has a yellow to reddish-brown color. The color is lighter when acid treating is employed. In 5 the latter case the resin is transparent in thin plates of say  $\frac{1}{2}$  centimeter thickness. It is soluble in petroleum naphtha, linseed oil, China wood oil, esters and benzol, and insoluble in water, lower alcohols and acetone.

10 The tar is often advantageously distilled in two steps. The first 60% is discarded and used as heating oil, and only the last 40% is used as starting material for the production of resins. Instead of the tar distillate other equally high 15 boiling petroleum oils such as for example the sulfur dioxide extract of a petroleum distillate which is rich in aromatic and/or unsaturated hydrocarbons may be used for producing resins, if it has a distillation range within approximately 20  $300^{\circ}$  F. to  $660^{\circ}$  F. under an absolute pressure of 1 mm. mercury. Other hydrocarbons such as distillates from an asphalt base crude, etc., may also be used as raw materials if they fall within the same approximate distillation range.

25 My process may be varied in different ways without departing from the spirit of the invention. Thus, for example, light colored resin may be prepared without using an acid treat. For this purpose the bottoms remaining in the de- 30 chlorinating still are dissolved in a small quantity of solvent such as ethylene dichloride, benzol, etc. A light paraffinic hydrocarbon such as petroleum ether, liquefied pentane or butane is then added to the solvent whereby the material dis- 35 solved, other than the resin, is precipitated and a fairly pure resin solution is obtained which does not need acid treatment. In another modification, still bottoms may be directly extracted by heating at atmospheric or higher pressure with 40 a light paraffinic hydrocarbon such as petroleum ether, butane or pentane. In this case again the resin goes into solution without appreciable amounts of contaminants. The resin solutions may be used either as such or the solvent may 45 be evaporated if a solid resin is required. The products obtained by my process may be characterized according to their source as resinified cracked tar oil or more generally as a resinified hydrocarbon distillate of petroleum origin.

50 Referring now to the drawing, 1 is a chlorinating vessel, 2 and 3 are the lines for introducing the distillate and the chlorine respectively, 4 the line for removing the evolved gases of chlorine, and hydrochloric acid, 5 a scrubber to remove the hydrochloric acid, and 6 a return line for the chlorine, 7 is the still for dechlorinating the product with an overhead line 8 and a bottoms draw-off line 9, which latter leads into the extractor 10. The extractor is provided with a line 11 for introducing the light naphtha or "Varsol", an agitator 12 and a draw-off line 13 leading to the filter press 14 to separate the naphtha-insoluble material. The solution is then either passed through acid treater 15 and neutralizer 16 60 to a still 17, or passed directly to the still 17. Valved lines 14a, 15a and 16a are provided for this purpose. The latter has the usual overhead

line and cooler 19 and the bottoms draw-off line 18 thru which the resin obtained as a residue is drawn off, cooled and sent to storage tank, (not shown).

The following example will serve to illustrate my process:

1,000 pounds of tar distillate from a cracking coil tar ( $10^{\circ}$  A. P. I.) representing the total overhead boiling up to  $660^{\circ}$  F. at 1 mm. pressure, was chlorinated until the percentage of combined chlorine reached 9.7%. The chlorinated distillate was then heated up to  $660^{\circ}$  F. in the still 7 provided with a condenser at atmospheric pressure, whereupon most of the chlorine was removed as hydrochloric acid. Then the distillate was subjected to a vacuum distillation under reduced pressure until a temperature corresponding to  $660^{\circ}$  F. at 1 mm. pressure was reached. 208 pounds of high softening point residue (S. P.  $282^{\circ}$  F. ball and ring method) was obtained in this way, which was extracted with light naphtha leaving an insoluble residue amounting to 75 pounds. After removal of the naphtha by distillation 133 pounds of light colored resin was obtained having a softening point of  $188^{\circ}$  F. (ball 100 and ring method).

This invention is not to be limited by any theory or the particular details given for purpose of illustration, but only by the following claims in which it is my intention to claim all novelty inherent in the process.

I claim:

1. A solid hydrocarbon resin produced by chlorination and dechlorination of a distillate boiling above about  $300^{\circ}$  F. at 1 mm. mercury absolute pressure, from a cracked petroleum tar, said resin being an unsaponifiable solid, clear, light yellow to reddish brown color, softening point above  $80^{\circ}$  F., soluble in petroleum naphtha, linseed oil and benzol and insoluble in water, lower alcohols and acetone.

2. Process for producing a resin, which comprises chlorinating a distillate, boiling within the approximate limits of 300 to  $660^{\circ}$  F. under an absolute pressure of 1 mm. mercury, from a cracked petroleum tar, heating the chlorinated distillate under a pressure below atmospheric to remove the chlorine and oily constituents therefrom as distillate, treating the remaining residue, substantially free from oily materials, with a selective solvent for resin, and separating the insoluble products from the solution containing the resin.

3. Process for producing a resin, which comprises chlorinating a distillate, boiling above about  $300^{\circ}$  F. at 1 mm. mercury absolute pressure, from a cracked petroleum tar, dechlorinating the chlorinated distillate by heating it to about  $660^{\circ}$  F. under vacuum, and extracting a resin from the dechlorinated residue product with a solvent.

4. Process according to claim 3, in which the hydrocarbon distillate treated boils within the approximate limits of 300 to  $660^{\circ}$  F. under an absolute pressure of 1 mm. mercury.

140

STEWART C. FULTON.